



US006063552A

# United States Patent [19]

Bourdelais et al.

[11] Patent Number: 6,063,552

[45] Date of Patent: May 16, 2000

[54] **PHOTOGRAPHIC CLEAR DISPLAY MATERIALS WITH BIAXIALLY ORIENTED POLYOLEFIN SHEET**

[75] Inventors: **Robert P. Bourdelais**, Pittsford; **Alphonse D. Camp**, Rochester; **Peter T. Aylward**, Hilton, all of N.Y.

[73] Assignee: **Eastman Kodak Company**, Rochester, N.Y.

[21] Appl. No.: 09/156,294

[22] Filed: Sep. 17, 1998

[51] Int. Cl.<sup>7</sup> G03C 1/795; G03C 1/93; G03C 7/30

[52] U.S. Cl. 430/363; 430/534; 430/536; 430/15; 430/939; 430/376

[58] Field of Search 430/15, 533, 534, 430/536, 939, 950, 502, 376

## [56] References Cited

### U.S. PATENT DOCUMENTS

|           |         |                |           |
|-----------|---------|----------------|-----------|
| 3,944,699 | 3/1976  | Mathews et al. | 428/220   |
| 4,187,113 | 2/1980  | Mathews et al. | 430/533   |
| 4,283,486 | 8/1981  | Aono et al.    | 430/505   |
| 4,632,869 | 12/1986 | Park et al.    | 428/315.5 |
| 4,758,462 | 7/1988  | Park et al.    | 428/213   |
| 4,900,654 | 2/1990  | Pollock et al. | 430/533   |

|           |         |                         |         |
|-----------|---------|-------------------------|---------|
| 4,912,333 | 3/1990  | Roberts et al. .        |         |
| 4,977,070 | 12/1990 | Winslow .....           | 430/510 |
| 5,055,371 | 10/1991 | Lee et al. .....        | 430/126 |
| 5,100,862 | 3/1992  | Harrison et al. .....   | 503/227 |
| 5,212,053 | 5/1993  | McSweeney et al. .....  | 430/503 |
| 5,244,861 | 9/1993  | Campbell et al. .....   | 430/201 |
| 5,387,501 | 2/1995  | Yajima et al. .....     | 430/533 |
| 5,389,422 | 2/1995  | Okazaki et al. .....    | 428/141 |
| 5,466,519 | 11/1995 | Shirakura et al. .....  | 430/538 |
| 5,866,282 | 2/1999  | Rourdelais et al. ..... | 430/536 |
| 5,888,643 | 3/1999  | Aylward et al. .....    | 430/536 |
| 5,888,681 | 3/1999  | Gula et al. .....       | 430/536 |

## FOREIGN PATENT DOCUMENTS

|              |         |                      |
|--------------|---------|----------------------|
| 0 662 633 A1 | 12/1995 | European Pat. Off. . |
| WO 94/04961  | 3/1994  | WIPO .               |

Primary Examiner—Richard L. Schilling  
Attorney, Agent, or Firm—Paul A. Leipold

## [57] ABSTRACT

The invention relates to a photographic element comprising a transparent polymer sheet, at least one layer of biaxially oriented polyolefin sheet and at least one image layer wherein said polymer sheet has a stiffness of between 20 and 100 millinewtons, and said biaxially oriented polyolefin sheet has a spectral transmission of at least 90% and a reflection density less than 10%.

16 Claims, No Drawings

**PHOTOGRAPHIC CLEAR DISPLAY  
MATERIALS WITH BIAXIALLY ORIENTED  
POLYOLEFIN SHEET**

**FIELD OF THE INVENTION**

This invention relates to photographic materials. In a preferred form it relates to base materials for photographic clear display.

**BACKGROUND OF THE INVENTION**

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters, and fine art photography. The desired attributes of a quality, high impact photographic display material are a slight blue density minimum, durability, sharpness, and flatness. Cost is also important, as display materials tend to be expensive compared with alternative display material technology, mainly lithographic images on paper. For display materials, traditional color paper is undesirable, as it suffers from a lack of durability for the handling, photo processing, and display of large format images. For clear display materials, a typical application is overhead projections of images and text during a business presentation.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. The formation of a suitably smooth surface would also improve image quality as the display material would have more apparent blackness as the reflective properties of the improved base are more specular than the prior materials. As the whites are whiter and the blacks are blacker, there is more range in between and, therefore, contrast is enhanced. It would be desirable if a more reliable and improved surface could be formed at less expense.

Prior art photographic reflective papers comprise a melt extruded polyethylene layer which also serves as a carrier layer for optical brightener and other whitener materials, as well as tint materials. It would be desirable if the optical brightener and tints, rather than being dispersed throughout the single melt extruded layer of polyethylene, could be concentrated nearer the surface where they would be more effective optically.

Prior art photographic clear display materials have light sensitive silver halide emulsions coated directly onto a gelatin coated clear polyester sheet. Clear photographic display materials are typically used as overhead and display materials with light boxes with diffuser screens. Diffusers are necessary to diffuse the light source used to backlight clear display materials. Without a diffuser, the light source would reduce the quality of the image. Since light sensitive silver halide emulsions tend to be yellow because of the gelatin used as a binder for photographic emulsions, minimum density areas of a developed image will tend to appear

yellow. A yellow white reduces the commercial value of a transmission display material because the imaging viewing public associates image quality with a white white. It would be desirable if a clear display material could have a more blue white, as a blue white is perceptually preferred by the public.

Prior art photographic display material uses polyester as a base for the support. Typically the polyester support is from 150 to 250  $\mu\text{m}$  thick to provide the required stiffness. A thinner base material would be lower in cost and allow for roll handling efficiency, as the rolls would weigh less and be smaller in diameter. It would be desirable to use a base material that had the required stiffness but was thinner to reduce cost and improve roll handling efficiency.

**PROBLEM TO BE SOLVED BY THE  
INVENTION**

There is a need for clear display materials that provide improved transmission of light while, at the same time, reducing the yellowness of the density minimum areas of the image.

**SUMMARY OF THE INVENTION**

It is an object of the invention to provide improved clear display materials.

It is another object to provide display materials that are lower in cost, as well as providing sharp durable images.

It is a further object to provide a clear display materials with a whiter density minimum.

These and other objects of the invention are accomplished by a photographic element comprising a transparent polymer sheet, at least one layer of biaxially oriented polyolefin sheet and at least one image layer wherein said polymer sheet has a stiffness of between 20 and 100 millinewtons, and said biaxially oriented polyolefin sheet has a spectral transmission of at least 90% and a reflection density less than 10%.

**ADVANTAGEOUS EFFECT OF THE  
INVENTION**

The invention provides whiter images by offsetting the yellowness of the light sensitive silver halide emulsion.

**DETAILED DESCRIPTION OF THE  
INVENTION**

The invention has numerous advantages over prior clear display materials and methods of imaging transmission display materials. The display materials of the invention provide very efficient diffusing of light while allowing the transmission of a high percentage of the light. The materials are low in cost, as the transparent polymer material sheet is thinner than in prior products. They are also lower in cost, as less gelatin is utilized and no antihillation layer is necessary. The display material of the invention will appear whiter to the observer than prior art materials which have a tendency to appear somewhat yellow, as the light sensitive silver halide emulsions used have a native yellowness. These and other advantages will be apparent from the detailed description below.

The terms as used herein, "top", "upper", "emulsion side", and "face" mean the side or toward the side of the photographic member bearing the imaging layers. The terms "bottom", "lower side", and "back" mean the side or toward the side of the photographic member opposite from the side bearing the photosensitive imaging layers or developed

image. The term as used herein, "transparent" or "clear" means the ability to pass radiation without significant deviation or absorption. For this invention, "transparent" or "clear" material is defined as a material that has a spectral transmission greater than 90%. For a photographic element, spectral transmission is the ratio of the transmitted power to the incident power and is expressed as a percentage as follows:  $T_{RGB}=10^{-D} * 100$  where D is the average of the red, green, and blue Status A transmission density response measured by an X-Rite model 310 (or comparable) photographic transmission densitometer.

For the clear display materials of this invention the layers of the biaxially oriented polyolefin sheet have levels of optical brightener and colorants adjusted to provide optimum light transmission properties. The functional optical properties for transmission display materials have been incorporated into the thin biaxially oriented polyolefin sheet. Colorants and optical brightener are added to a thin layer of the biaxially oriented sheet of this invention to offset the native yellowness of the photographic imaging layers. The biaxially oriented polyolefin sheet is laminated to a transparent polymer base for stiffness for efficient image processing, as well as product handling and display. An important aspect of this invention is the incorporation of a low level of microvoiding to diffuse some of the backlighting source. For projection images, this allows for efficient projection of the image onto a display surface, yet provides some level of backlight diffusion which reduces undesirable glare from the projection light source.

Any suitable biaxially oriented polyolefin sheet may be utilized for the sheet on the top side of the laminated base of the invention. The core of the preferred composite sheet should be from 15 to 95% of the total thickness of the sheet, preferably from 30 to 85% of the total thickness. The skin(s) should thus be from 5 to 85% of the sheet, preferably from 15 to 70% of the thickness.

The total thickness of the composite sheet can range from 12 to 100  $\mu\text{m}$ , preferably from 20 to 70  $\mu\text{m}$ . Below 20  $\mu\text{m}$ , the microvoided sheets may not be thick enough to minimize any inherent nonplanarity in the support and would be more difficult to manufacture. At thickness higher than 70  $\mu\text{m}$ , little improvement in either surface smoothness or mechanical properties is seen, and so there is little justification for the further increase in cost for extra materials.

For the biaxially oriented sheets on the top side toward the emulsion, suitable classes of thermoplastic polymers for the biaxially oriented sheet and the core matrix-polymer of the preferred composite sheet comprise polyolefins. Suitable polyolefins include polypropylene, polyethylene, polymethylpentene, polystyrene, polybutylene, and mixtures thereof. Polyolefin copolymers, including copolymers of propylene and ethylene such as hexene, butene, and octene are also useful. Polypropylene is preferred, as it is low in cost and has desirable strength properties.

The skin layers of the composite sheet can be made of the same polymeric materials as listed above for the core matrix. The composite sheet can be made with skin(s) of the same polymeric material as the core matrix, or it can be made with skin(s) of different polymeric composition than the core matrix.

The total thickness of the topmost skin layer or exposed surface layer should be between 0.20  $\mu\text{m}$  and 1.5  $\mu\text{m}$ , preferably between 0.5 and 1.0  $\mu\text{m}$ . Below 0.5  $\mu\text{m}$  any inherent nonplanarity in the coextruded skin layer may result in unacceptable color variation. At skin thickness greater than 1.0  $\mu\text{m}$ , there is a reduction in the photographic optical

properties such as image resolution. At thickness greater than 1.0  $\mu\text{m}$ , there is also a greater material volume to filter for contamination such as clumps, poor color pigment dispersion, or contamination. Low density polyethylene with a density of 0.88 to 0.94 g/cc is the preferred material for the top skin because current emulsion formulation adheres well to low density polyethylene compared to other materials such as polypropylene and high density polyethylene.

Addenda may be added to the topmost skin layer to change the color of the imaging element. For photographic use, a white base with a slight bluish tinge is preferred. The addition of the slight bluish tinge may be accomplished by any process which is known in the art including the machine blending of color concentrate prior to extrusion and the melt extrusion of blue colorants that have been preblended at the desired blend ratio. Colored pigments that can resist extrusion temperatures greater than 320° C. are preferred, as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, Irgalite organic blue pigments, and pigment Blue 60.

In a preferred embodiment of this invention it has been found that a very thin coating (0.2 to 1.5  $\mu\text{m}$ ) on the surface immediately below the emulsion layer can be made by coextrusion and subsequent stretching in the width and length direction. It has been found that this layer is, by nature, extremely accurate in thickness and can be used to provide all the color corrections which are usually distributed throughout the thickness of the sheet between the emulsion and the paper base. This topmost layer is so efficient that the total colorants needed to provide a correction are less than one-half the amount needed if the colorants are dispersed throughout thickness. Colorants are often the cause of spot defects due to clumps and poor dispersions. Spot defects, which decrease the commercial value of images, are improved with this invention because less colorant is used, and high quality filtration to clean up the colored layer is much more feasible since the total volume of polymer with colorant is only typically 2 to 10 percent of the total polymer between the base paper and the photosensitive layer.

Addenda may be added to the biaxially oriented sheet of this invention so that when the biaxially oriented sheet is viewed by the intended audience, the imaging element emits light in the visible spectrum when exposed to ultraviolet radiation. Emission of light in the visible spectrum allows for the support to have a desired background color in the presence of ultraviolet energy. This is particularly useful when images are backlit with a light source that contains ultraviolet energy and may be used to optimize image quality for transmission display applications.

Addenda known in the art to emit visible light in the blue spectrum are preferred. Consumers generally prefer a slight blue tint to white defined as a negative  $b^*$  compared to a white white defined as a  $b^*$  within one  $b^*$  unit of zero.  $b^*$  is the measure of yellow/blue in CIE space. A positive  $b^*$  indicates yellow, while a negative  $b^*$  indicates blue. The addition of addenda that emits in the blue spectrum allows for tinting the support without the addition of colorants which would decrease the whiteness of the image. The preferred emission is between 1 and 5 delta  $b^*$  units. Delta  $b^*$  is defined as the  $b^*$  difference measured when a sample is illuminated ultraviolet light source and a light source

without any significant ultraviolet energy. Delta b\* is the preferred measure to determine the net effect of adding an optical brightener to the top biaxially oriented sheet of this invention. Emissions less than 1 b\* unit cannot be noticed by most customers; therefore is it not cost effective to add such a small amount of optical brightener to the biaxially oriented sheet. An emission greater than 5 b\* units would interfere with the color balance of the prints, making the whites appear too blue for most consumers.

The preferred addenda for the emission of blue light is an optical brightener. An optical brightener is a substantially colorless, fluorescent, organic compound that absorbs ultraviolet light and emits it as visible blue light. Examples include but are not limited to derivatives of 4,4'-diaminostilbene-2,2'-disulfonic acid, coumarin derivatives such as 4-methyl-7-diethylaminocoumarin, 1-4-Bis (O-Cyanostyryl) Benzol and 2-Amino-4-Methyl Phenol. An unexpected desirable feature of this invention is the efficient use of optical brightener. Because the ultraviolet source for a transmission display material is on the opposite side of the image, the ultraviolet light intensity is not reduced by ultraviolet filters common to imaging layers. The result is that less optical brightener is required to achieve the desired background color.

The optical brightener may be added to any layer in the multilayer coextruded biaxially oriented polyolefin sheet. The preferred location is adjacent to or in the exposed surface layer of said sheet. This allows for the efficient concentration of optical brightener which results in less optical brightener being used when compared to traditional photographic supports. When the desired weight % loading of the optical brightener begins to approach the concentration at which the optical brightener migrates to the surface of the support forming crystals in the imaging layer, the addition of optical brightener into the layer adjacent to the exposed layer is preferred. When optical brightener migration is a concern as with light sensitive silver halide imaging systems, the preferred exposed layer comprised polyethylene. In this case, the migration from the layer adjacent to the exposed layer is significantly reduced, allowing for much higher optical brightener levels to be used to optimize image quality. Locating the optical brightener in the layer adjacent to the upper exposed layer allows for a less expensive optical brightener to be used as the upper exposed layer, which is substantially free of optical brightener, and which prevents significant migration of the optical brightener. Another preferred method to reduce unwanted optical brightener migration is to use polypropylene for the layer adjacent to the exposed surface. Since optical brightener is more soluble in polypropylene than polyethylene, the optical brightener is less likely to migrate from polypropylene.

A biaxially oriented polyolefin sheet substantially free of white pigments is preferred. White pigments such as TiO<sub>2</sub> added to the polyolefin sheets tend to scatter light and reduce the spectral transmission of the support. Light scattering and a reduction in spectral transmission are undesirable for clear display materials.

The preferred spectral transmission of the biaxially oriented polyolefin sheet of this invention is at least 90%. Spectral transmission is the amount of light energy that is transmitted through a material. For a photographic element, spectral transmission is the ratio of the transmitted power to the incident power and is expressed as a percentage as follows: T<sub>RGB</sub>=10<sup>-D</sup> \* 100 where D is the average of the red, green, and blue Status A transmission density response measured by an X-Rite model 310 (or comparable) photographic transmission densitometer. The higher the

transmission, the less opaque the material. For a clear display material, the quality of the image is related to the amount of light transmitted through the image. A clear display image with a low amount of spectral transmission does not allow sufficient illumination of the image causing a perceptual loss in image quality. A transmission image with a spectral transmission of less than 85% is unacceptable for a clear display material, as the quality of the image cannot match prior art clear display materials.

The most preferred spectral transmission density for the biaxially oriented sheets of this invention is between 92% and 98%. This range allows for optimization of transmission properties to create a clear display material that can be used as an overhead or display material in combination with a light box and diffuser screen.

A reflection density less than 10% for the biaxially oriented sheet of this invention is preferred. Reflection density is the amount of light energy reflecting from the image to an observer's eye. Reflection density is measured by 0°/45° geometry Status A red/green/blue response using an X-Rite model 310 (or comparable) photographic transmission densitometer. A sufficient amount of reflective light energy is required to diffuse the backlighting source. A reflection density greater than 10% is unacceptable for a clear display material and does not match the quality of prior art clear display materials.

A biaxially oriented sheet of this invention which has a limited amount of microvoiding in the core may also be used. The microvoided core adds whiteness to the imaging support, allowing for diffusion of the light source while allowing for sufficient transmission of light. The voided core is an excellent diffuser of light and has substantially less light scatter than white pigments such as TiO<sub>2</sub>. Less light scatter improves the quality of the transmitted image. Combining the image quality advantages of a microvoided core with a material, which absorbs ultraviolet energy and emits light in the visible spectrum, allows for the unique optimization of image quality as the image support can have a tint when exposed to ultraviolet energy, yet retain excellent whiteness when the image is viewed using lighting that does not contain significant amounts of ultraviolet energy such as indoor lighting. A low level of voiding of the biaxially oriented sheet of this invention should be used to avoid reducing the % transmission below 90%.

The coextrusion, quenching, orienting, and heat setting of these biaxially oriented polyolefin composite sheets may be effected by any process which is known in the art for producing oriented sheet, such as by a flat sheet process or a bubble or tubular process. The flat sheet process involves extruding the blend through a slit die and rapidly quenching the extruded web upon a chilled casting drum so that the core matrix polymer component of the sheet and the skin component(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. A stretching ratio, defined as the final length divided by the original length for sum of the machine and cross directions, of at least 10 to 1 is preferred. After the sheet has been stretched, it is heat set by heating to a temperature sufficient to crystallize or anneal the polymers, while restraining to some degree the sheet against retraction in both directions of stretching.

The composite sheet, while described as having preferably at least two layers, may also be provided with addi-

tional layers that may serve to change the properties of the biaxially oriented sheet. Biaxially oriented sheets could be formed with surface layers that would provide an improved adhesion, or improved look to the support and photographic element. The biaxially oriented extrusion could be carried out with as many as 10 layers if desired to achieve some particular desired property.

These composite sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photosensitive layers. Examples of this would be acrylic coatings for printability and coating polyvinylidene chloride for heat seal properties. Further examples include flame, plasma, or corona discharge treatment to improve printability or adhesion.

The structure of a preferred biaxially oriented sheet where the exposed surface layer is adjacent to the imaging layer is as follows:

Polyethylene skin with blue pigments

Polypropylene

The transparent support to which the microvoided composite sheets and biaxially oriented sheets are laminated for the laminated support of the photosensitive silver halide layer may be any material with the desired transmission and stiffness properties. Photographic elements of the invention can be prepared on any suitable synthetic paper such as polystyrene, ceramics, synthetic high molecular weight sheet materials such as polyalkyl acrylates or methacrylates, polystyrene, polyamides such as nylon, sheets of semisynthetic high molecular weight materials such as cellulose nitrate, cellulose acetate butyrate, and the like; homo and copolymers of vinyl chloride, poly(vinylacetal), polycarbonates, homo and copolymers of olefins such as polyethylene and polypropylene, and the like.

Polyester sheets are particularly advantageous because they provide excellent strength and dimensional stability. Such polyester sheets are well known, widely used, and typically prepared from high molecular weight polyesters prepared by condensing a dihydric alcohol with a dibasic saturated fatty acid or derivative thereof.

Suitable dihydric alcohols for use in preparing such polyesters are well known in the art and include any glycol wherein the hydroxyl groups are on the terminal carbon atom and contain from 2 to 12 carbon atoms such as, for example, ethylene glycol, propylene glycol, trimethylene glycol, hexamethylene glycol, decamethylene glycol, dodecamethylene glycol, 1,4-cyclohexane, dimethanol, and the like.

Suitable dibasic acids useful for the preparation of polyesters include those containing from 2 to 16 carbon atoms such as adipic acid, sebatic acid, isophthalic acid, terephthalic acid, and the like. Alkyl esters of acids such as those listed above can also be employed. Other alcohols and acids, as well as polyesters prepared therefrom and the preparation of the polyesters, are described in U.S. Pat. No. 2,720,503 and 2,901,466 which are hereby incorporated herein by reference. Polyethylene terephthalate is preferred.

Polyester support thickness in any direction (machine direction or cross direction) can range from about 15 millinewtons to 100 millinewtons. The preferred stiffness is between 20 and 100 millinewtons. Polyester stiffness less than 15 millinewtons does not provide the required stiffness for display materials in that they will be difficult to handle and do not lay flat for optimum viewing. Polyester stiffness

greater than 100 millinewtons begins to exceed the stiffness limit for processing equipment and has no performance benefit for the display materials.

Generally polyester films supports are prepared by melt extruding the polyester through a slit die, quenching to the amorphous state, orienting by machine and cross direction stretching, and heat setting under dimensional restraint. The polyester film can also be subjected to a heat relaxation treatment to improve dimensional stability and surface smoothness.

The polyester film will typically contain a subbing, undercoat, or primer layer on both sides of the polyester film. Subbing layers used to promote adhesion of coating compositions to the support are well known in the art, and any such material can be employed. Some useful compositions for this purpose include interpolymers of vinylidene chloride such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627,088; 2,698,240; 2,943,937; 3,143,421; 3,201,249; 3,271,178; 3,443,950; and 3,501,301. The polymeric subbing layer is usually overcoated with a second subbing layer comprised of gelatin, typically referred to as gel sub.

The base also may be a microvoided polyethylene terephthalate such as disclosed in U.S. Pat. Nos. 4,912,333; 4,994,312; and 5,055,371.

A transparent polymer base free of  $TiO_2$  is preferred because the  $TiO_2$  in the transparent polymer reduces the light transmission and will tend to scatter light, thereby reducing the quality of the image. The  $TiO_2$  pigmented transparent polymer also is expensive because the  $TiO_2$  must be dispersed into the entire thickness, typically from 100 to 180  $\mu m$ . The  $TiO_2$  also gives the transparent polymer support a slight yellow tint which is undesirable for a photographic display material. For use as a photographic reflective display material, a transparent polymer support containing  $TiO_2$  must also be tinted blue to offset the yellow tint of the polyester causing a loss in desired whiteness and adding cost to the display material. Concentration of the white pigment in the polyolefin layer allows for efficient use of the white pigment which improves image quality and reduces the cost of the imaging support.

When using a polyester base, it is preferable to extrusion laminate the microvoided composite sheets to the polyester base using a polyolefin resin. Extrusion laminating is carried out by bringing together the biaxially oriented sheets of the invention and the polyester base with application of a melt extruded adhesive between the polyester sheets and the biaxially oriented polyolefin sheets followed by their being pressed in a nip such as between two rollers. The melt extruded adhesive may be applied to either the biaxially oriented sheets or the polyester sheet prior to their being brought into the nip. In a preferred form the adhesive is applied into the nip simultaneously with the biaxially oriented sheets and the polyester sheet. The adhesive used to adhere the biaxially oriented polyolefin sheet to the polyester base may be any suitable material that does not have a harmful effect upon the photographic element. A preferred material is metallocene catalyzed ethylene plastomers that are melt extruded into the nip between the paper and the biaxially oriented sheet. Metallocene catalyzed ethylene plastomers are preferred because they are easily melt extruded, adhere well to biaxially oriented polyolefin sheets of this invention, and adhere well to gelatin sub polyester support of this invention.

The structure of a preferred clear display support where the imaging layers are applied to the biaxially oriented polyolefin sheet is as follows:

Biaxially oriented polyolefin sheet  
Metallocene catalyzed ethylene plastomer  
Gelatin coating

Polyester base  
Gelatin coating

As used herein, the phrase "photographic element" is a material that utilizes photosensitive silver halide in the formation of images. The photographic elements can be single color elements, black-and-white, or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

For the clear display material of this invention, at least one imaging layer containing silver halide and a dye forming coupler located on the top side of the clear support of this invention is preferred.

The photographic emulsions useful for this invention are generally prepared by precipitating silver halide crystals in a colloidal matrix by methods conventional in the art. The colloid is typically a hydrophilic film forming agent such as gelatin, alginic acid, or derivatives thereof.

The crystals formed in the precipitation step are washed and then chemically and spectrally sensitized by adding spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sensitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, curtain coating, and extrusion coating.

The silver halide emulsions utilized in this invention may be comprised of any halide distribution. Thus, they may be comprised of silver chloride, silver bromide, silver bromochloride, silver chlorobromide, silver iodochloride, silver iodobromide, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride, and optimally greater than about 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H. James, Macmillan Publishing Company, Inc., 1977, pages 151-152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitization include ascorbic acid derivatives; tin compounds; polyamine compounds; and thiourea dioxide-based compounds described in U.S. Pat. Nos. 2,487,850; 2,512,925; and British Patent 789,823. Specific examples of reduction sensitizers or conditions, such as dimethylamineborane, stannous chloride, hydrazine, high pH (pH 8-11) and low pAg (pAg 1-7) ripening are discussed by S. Collier in *Photographic Science and Engineering*, 23, 113 (1979). Examples of processes for preparing intentionally reduction sensitized silver halide emulsions are described in EP 0 348 934 A1 (Yamashita), EP 0 369 491 (Yamashita), EP 0 371 388 (Ohashi), EP 0 396 424 A1 (Takada), EP 0 404 142 A1 (Yamada), and EP 0 435 355 A1 (Makino).

The photographic elements of this invention may use emulsions doped with Group VIII metals such as iridium, rhodium, osmium, and iron as described in *Research Disclosure*, September 1994, Item 36544, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," *Photographic Science and Engineering*, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in *The British Journal of Photography Annual*, 1982, pages 201-203.

A typical multicolor photographic element of the invention comprises the invention laminated support bearing a cyan dye image-forming unit comprising at least one red-sensitive silver halide emulsion layer having associated

## 11

therewith at least one cyan dye-forming coupler; a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black-and-white photographic print elements.

The invention may be utilized with the materials disclosed in *Research Disclosure*, 40145 of September 1997. The invention is particularly suitable for use with the materials of the color paper examples of sections XVI and XVII. The couplers of section II are also particularly suitable. The Magenta I couplers of section II, particularly M-7, M-10, M-11, and M-18 set forth below are particularly desirable.

## 12

light. Halation can be greatly reduced or eliminated by absorbing the light transmitted by the emulsion or piped by the support. Three methods of providing halation protection are (1) coating an antihalation undercoat which is either dye 5 gelatin or gelatin containing gray silver between the emulsion and the support, (2) coating the emulsion on a support that contains either dye or pigments, and (3) coating the emulsion on a transparent support that has a dye to pigment 10 a layer coated on the back. The absorbing material contained in the antihalation undercoat or antihalation backing is removed by processing chemicals when the photographic element is processed. The dye or pigment within the support is permanent and generally is not preferred for the instant invention. In the instant invention, it is preferred that the 15 antihalation layer be formed of gray silver which is coated on the side furthest from the top and removed during processing. By coating furthest from the top on the back surface, the antihalation layer is easily removed, as well as



M-7



M-10



M-11



M-18

The element of the invention may contain an antihalation layer. A considerable amount of light may be diffusely transmitted by the emulsion and strike the back surface of the support. This light is partially or totally reflected back to the emulsion and reexposed it at a considerable distance from the initial point of entry. This effect is called halation because it causes the appearance of halos around images of bright objects. Further, a transparent support also may pipe

60 allowing exposure of the duplitized material from only one side. If the material is not duplitized, the gray silver could be coated between the support and the top emulsion layers where it would be most effective. The problem of halation is 65 minimized by coherent collimated light beam exposure, although improvement is obtained by utilization of an antihalation layer even with collimated light beam exposure.

In order to successfully transport display materials of the invention, the reduction of static caused by web transport through manufacturing and image processing is desirable. Since the light sensitive imaging layers of this invention can be fogged by light from a static discharge accumulated by the web as it moves over conveyance equipment such as rollers and drive nips, the reduction of static is necessary to avoid undesirable static fog. The polymer materials of this invention have a marked tendency to accumulate static charge as they contact machine components during transport. The use of an antistatic material to reduce the accumulated charge on the web materials of this invention is desirable. Antistatic materials may be coated on the web materials of this invention and may contain any known materials in the art which can be coated on photographic web materials to reduce static during the transport of photographic paper. Examples of antistatic coatings include conductive salts and colloidal silica. Desirable antistatic properties of the support materials of this invention may also be accomplished by antistatic additives which are an integral part of the polymer layer. Incorporation of additives that migrate to the surface of the polymer to improve electrical conductivity include fatty quaternary ammonium compounds, fatty amines, and phosphate esters. Other types of antistatic additives are hygroscopic compounds such as polyethylene glycols and hydrophobic slip additives that reduce the coefficient of friction of the web materials. An antistatic coating applied to the opposite side of the image layer or incorporated into the backside polymer layer is preferred. The backside is preferred because the majority of the web contact during conveyance in manufacturing and photoprocessing is on the backside. The preferred surface resistivity of the antistat coat at 50% RH is less than  $10^{13}$  ohm/square. A surface resistivity of the antistat coat at 50% RH is less than  $10^{13}$  ohm/square has been shown to sufficiently reduce static fog in manufacturing and during photoprocessing of the image layers.

The invention photographic imaging members may contain matte beads to help aid in stacking, winding, and unwinding of the photographic members without damage. Matte beads are known in the formation of prior display imaging materials. The matte beads may be applied on the top or bottom of the imaging members. Generally, if applied on the emulsion side, the beads are below the surface protective layer (SOC).

In the following Table, reference will be made to (1) *Research Disclosure*, December 1978, Item 17643, (2) *Research Disclosure*, December 1989, Item 308119, and (3) *Research Disclosure*, September 1996, Item 38957, all published by Kenneth Mason Publications, Ltd., Dudley Annex, 12a North Street, Emsworth, Hampshire PO10 7DQ, ENGLAND. The Table and the references cited in the Table are to be read as describing particular components suitable for use in the elements of the invention. The Table and its cited references also describe suitable ways of preparing, exposing, processing and manipulating the elements, and the images contained therein.

-continued

| Reference | Section         | Subject Matter                                                        |
|-----------|-----------------|-----------------------------------------------------------------------|
| 5         | 3               | A & B                                                                 |
| 1         | III, IV         | Chemical sensitization and spectral sensitization/                    |
| 2         | III, IV         | desensitization                                                       |
| 3         | IV, V           | UV dyes, optical brighteners, luminescent dyes                        |
| 10        | 1               |                                                                       |
| 2         | V               |                                                                       |
| 3         | VI              |                                                                       |
| 1         | VI              |                                                                       |
| 2         | VI              | Antifoggants and stabilizers                                          |
| 3         | VII             |                                                                       |
| 1         | VIII            |                                                                       |
| 2         | VIII, XIII, XVI | Absorbing and scattering materials; Antistatic layers; matting agents |
| 15        | 3               | VIII, IX C & D                                                        |
| 1         | VII             | Image-couplers and image-modifying couplers; Dye                      |
| 2         | VII             | stabilizers and hue modifiers                                         |
| 3         | X               |                                                                       |
| 1         | XVII            |                                                                       |
| 2         | XVII            | Supports                                                              |
| 3         | XV              |                                                                       |
| 3         | XI              | Specific layer arrangements                                           |
| 3         | XII, XIII       | Negative working emulsions; Direct positive emulsions                 |
| 20        | 2               | Exposure                                                              |
| 25        | 3               |                                                                       |
| 1         | XIX, XX         | Chemical processing; Developing agents                                |
| 2         | XIX, XX, XXII   |                                                                       |
| 3         | XVIII, XIX, XX  |                                                                       |
| 30        | 3               | Scanning and digital processing procedures                            |

The photographic elements can be exposed with various forms of energy which encompass the ultraviolet, visible, and infrared regions of the electromagnetic spectrum, as well as with electron beam, beta radiation, gamma radiation, X ray, alpha particle, neutron radiation, and other forms of corpuscular and wavelike radiant energy in either noncoherent (random phase) forms or coherent (in phase) forms, as produced by lasers. When the photographic elements are intended to be exposed by X rays, they can include features found in conventional radiographic elements.

The photographic elements are preferably exposed to actinic radiation, typically in the visible region of the spectrum, to form a latent image, and then processed to form a visible image, preferably by other than heat treatment. Processing is preferably carried out in the known RA-4™ (Eastman Kodak Company) Process or other processing systems suitable for developing high chloride emulsions.

The following examples illustrate the practice of this invention. They are not intended to be exhaustive of all possible variations of the invention. Parts and percentages are by weight unless otherwise indicated.

## EXAMPLES

## Example 1

The following prior art clear display material was used as a control for the invention in this example:

60 Kodak DuraClear (Eastman Kodak Co.), is a one side color silver halide coated polyester support that is 180  $\mu\text{m}$  thick. The support is a clear gel coated photographic grade polyester.

The following example of the invention was prepared by 65 laminating photographic clear display material by extrusion laminating the following biaxially oriented sheet to top side of a photographic grade polyester base:

| Reference | Section                        | Subject Matter                                                                                    |
|-----------|--------------------------------|---------------------------------------------------------------------------------------------------|
| 1         | I, II                          | Grain composition,                                                                                |
| 2         | I, II, IX, X, XI, XII, XIV, XV | morphology and preparation. Emulsion preparation including hardeners, coating aids, addenda, etc. |
|           | I, II, IX                      |                                                                                                   |

## Top Sheet (Emulsion side):

A composite biaxially oriented sheet consisting of 2 layers identified as **L1** and **L2**. **L1** is the thin colored 0.75  $\mu\text{m}$  polyethylene layer on the outside of the package to which the photosensitive silver halide layer was attached. **L2** is a 18  $\mu\text{m}$  polypropylene layer.

## Photographic grade polyester base:

A polyethylene terephthalate base 110  $\mu\text{m}$  thick that was transparent and gelatin sub on both sides of the base. The polyethylene terephthalate base had a stiffness of 30 millinewtons in the machine direction and 40 millinewtons in the cross direction.

The top sheet was melt extrusion laminated to the photographic grade polyester base using an metallocene catalyzed ethylene plastomer (SLP 9088) manufactured by Exxon Chemical Corp. The metallocene catalyzed ethylene plastomer had a density of 0.900 g/cc and a melt index of 14.0.

Coating format 1 was utilized to prepare photographic reflective material was coated on the **L1** polyethylene layer on the top biaxially oriented sheet.

|         | Coating Format 1           | Laydown mg/m <sup>2</sup> |
|---------|----------------------------|---------------------------|
| Layer 1 | <u>Blue Sensitive</u>      |                           |
|         | Gelatin                    | 1300                      |
|         | Blue sensitive silver      | 200                       |
|         | Y-1                        | 440                       |
|         | ST-1                       | 440                       |
|         | S-1                        | 190                       |
| Layer 2 | <u>Interlayer</u>          |                           |
|         | Gelatin                    | 650                       |
|         | SC-1                       | 55                        |
|         | S-1                        | 160                       |
| Layer 3 | <u>Green Sensitive</u>     |                           |
|         | Gelatin                    | 1100                      |
|         | Green sensitive silver     | 70                        |
|         | M-1                        | 270                       |
|         | S-1                        | 75                        |
|         | S-2                        | 32                        |
|         | ST-2                       | 20                        |
|         | ST-3                       | 165                       |
|         | ST-4                       | 530                       |
| Layer 4 | <u>UV Interlayer</u>       |                           |
|         | Gelatin                    | 635                       |
|         | UV-1                       | 30                        |
|         | UV-2                       | 160                       |
|         | SC-1                       | 50                        |
|         | S-3                        | 30                        |
|         | S-1                        | 30                        |
| Layer 5 | <u>Red Sensitive Layer</u> |                           |
|         | Gelatin                    | 1200                      |
|         | Red sensitive silver       | 170                       |
|         | C-1                        | 365                       |
|         | S-1                        | 360                       |
|         | UV-2                       | 235                       |
|         | S-4                        | 30                        |
|         | SC-1                       | 3                         |
| Layer 6 | <u>UV Overcoat</u>         |                           |
|         | Gelatin                    | 440                       |
|         | UV-1                       | 20                        |
|         | UV-2                       | 110                       |
|         | SC-1                       | 30                        |
|         | S-3                        | 20                        |
|         | S-1                        | 20                        |
| Layer 7 | <u>SOC</u>                 |                           |
|         | Gelatin                    | 490                       |
|         | SC-1                       | 17                        |

-continued

| Coating Format 1 | Laydown mg/m <sup>2</sup> |
|------------------|---------------------------|
| SiO <sub>2</sub> | 200                       |
| Surfactant       | 2                         |

## APPENDIX

Y-1



25 ST-1=N-tert-butylacrylamide/n-butyl acrylate copolymer (50:50)

S-1=dibutyl phthalate

SC-1



M-1



S-2=diundecyl phthalate

ST-2



ST-3



ST-4





S-3=1,4-Cyclohexyldimethylene bis(2-ethylhexanoate)



S-4=2-(2-Butoxyethoxy)ethyl acetate



The bending stiffness of the polyester base and the laminated display material support was measured by using the Lorentzen and Wettre stiffness tester, Model 16D. The output from this instrument is force, in millinewtons, required to bend the cantilevered, unclasped end of a sample 20 mm long and 38.1 mm wide at an angle of 15 degrees from the unloaded position. In this test the stiffness in both the machine direction and cross direction of the polyester base was compared to the stiffness of the base laminated with the top biaxially oriented sheet of this example. The results are presented in Table 3.

UV-1

|                           | Machine Direction<br>Stiffness<br>(millinewtons) | Cross Direction<br>Stiffness<br>(millinewtons) |
|---------------------------|--------------------------------------------------|------------------------------------------------|
| 5<br>Before<br>Lamination | 33                                               | 23                                             |
| 10<br>After<br>Lamination | 87                                               | 80                                             |

UV-2

The data above in Table 3 show the significant increase in stiffness of the polyester base after lamination with a biaxially oriented polymer sheet. This result is significant in that prior art materials, in order to provide the necessary stiffness, used polyester bases that were much thicker (between 150 and 256  $\mu\text{m}$ ) compared to the 110  $\mu\text{m}$  polyester base used in this example. At equivalent stiffness, the significant increase in stiffness after lamination allows for a thinner polyester base to be used compared to prior art materials, thus reducing the cost of the clear display support. Further, a reduction in clear display material thickness allows for a reduction in material handling costs, as rolls of thinner material weigh less and are smaller in roll diameter.

The clear display material was processed as a minimum density. The display support was measured for status A density using an X-Rite Model 310 photographic densitometer. Spectral transmission is calculated from the Status A density readings and is the ratio of the transmitted power to the incident power and is expressed as a percentage as follows:  $T_{RGB}=10^{-D} * 100$  where D is the average of the red, green, and blue Status A transmission density response. The display materials were also measured for  $L^*$ ,  $a^*$ , and  $b^*$  using a Spectroguard spectrophotometer, CIE system, using illuminant D6500. The results are presented in Table 2 below.

TABLE 2

|    | Measure         | Invention | Control |
|----|-----------------|-----------|---------|
| 40 | % Transmission  | 94%       | 85%     |
| 1  | CIE D6500 $L^*$ | 93.4      | 93.22   |
|    | CIE D6500 $a^*$ | -0.46     | -0.089  |
|    | CIE D6500 $b^*$ | 1.24      | 2.37    |

45 The clear display support coated on the top side with the light sensitive silver halide coating format of this example exhibits all the properties needed for a photographic display material that can function as a clear display material. Further, the photographic transmission display material of 50 this example has many advantages over prior art photographic display materials. The nonvoided layers have levels of optical brightener and colorants adjusted to provide an improved minimum density position compared to prior art transmission display materials as the invention was able to overcome the native yellowness of the processed emulsion layers ( $b^*$  for the invention was 1.24 compared to the  $b^*$  of 2.37 for the control material). For clear display materials, a blue white is more perceptually preferred than a yellow white, creating a higher quality image for the invention 55 compared to the control material.

60 The 94% transmission for the invention provides a superior clear image as the invention allows for a high quality projection of the image. The  $a^*$  and  $L^*$  for the invention are consistent with a high quality transmission display materi-

als. Finally the invention would be lower in cost over prior art materials as a transparent 100  $\mu\text{m}$  polyester base was used in the invention compared to a typical 180 to 250  $\mu\text{m}$  polyester for prior art photographic clear display materials.

The invention has been described in detail with particular reference to preferred embodiments thereof, but it will be understood that variations and modifications can be effected within the spirit and scope of the invention.

What is claimed is:

1. A photographic element comprising a transparent polymer sheet, at least one layer of biaxially oriented polyolefin sheet and at least one image layer wherein said polymer sheet has a stiffness of between 20 and 100 millinewtons, and said biaxially oriented polyolefin sheet has a spectral transmission of at least 90% and a reflection density less than 10%. 10
2. The photographic element of claim 1 wherein said reflection density is between 3 and about 8%. 15
3. The photographic element of claim 1 wherein said biaxially oriented polyolefin sheet has an integral layer of polyethylene on the top of said sheet. 20
4. The photographic element of claim 1 wherein said spectral transmission is between 92 and 98%. 25
5. The photographic element of claim 1 wherein said transparent polymer sheet is substantially free of pigment. 25
6. The photographic element of claim 1 wherein said at least one image layer comprises at least one imaging layer containing silver halide and a dye forming coupler located on the top side of said imaging element. 30
7. The photographic element of claim 1 wherein said biaxially oriented polyolefin sheet is substantially free of white pigments. 30

8. The photographic element of claim 1 wherein said polymer sheet comprises polyester.

9. A method of imaging comprising providing an photographic element comprising a transparent polymer sheet, at least one layer of biaxially oriented polyolefin sheet and at least one image layer comprising silver halide and a dye forming coupler, wherein said polymer sheet has a stiffness of between 20 and 100 millinewtons, and said biaxially oriented polyolefin sheet has a spectral transmission of at least 90% and a reflection density less than 10%, exposing said image layer, and developing an image.

10. The method of claim 9 wherein said reflection density is between 3 and about 8%.

11. The method of claim 9 wherein said biaxially oriented polyolefin sheet has an integral layer of polyethylene on the top of said sheet.

12. The method of claim 9 wherein said spectral transmission is between 92 and 98%.

13. The method of claim 9 wherein said transparent polymer sheet is substantially free of pigment.

14. The method of claim 9 wherein said at least one image layer comprises at least one imaging layer containing silver halide and a dye forming coupler located on the top side of said imaging element.

15. The method of claim 9 wherein said biaxially oriented polyolefin sheet is substantially free of white pigments.

16. The method of claim 9 wherein said polymer sheet comprises polyester.

\* \* \* \* \*